



US012351983B2

(12) **United States Patent**  
Ankeny et al.

(10) **Patent No.:** US 12,351,983 B2  
(45) **Date of Patent:** Jul. 8, 2025

(54) **PRETREATMENT METHODS FOR COTTON TEXTILE WASTE FABRIC**

(71) Applicants: **NORTH CAROLINA STATE UNIVERSITY**, Raleigh, NC (US); **Cotton Incorporated**, Cary, NC (US)

(72) Inventors: **Mary Ann Ankeny**, Raleigh, NC (US); **Matthew J. Farrell**, Apex, NC (US); **Ronalds Gonzalez**, Apex, NC (US); **Hasan Jameel**, Raleigh, NC (US)

(73) Assignees: **NORTH CAROLINA STATE UNIVERSITY**, Raleigh, NC (US); **Cotton Incorporated**, Cary, NC (US)

(\*) Notice: Subject to any disclaimer, the term of this patent is extended or adjusted under 35 U.S.C. 154(b) by 267 days.

(21) Appl. No.: **18/062,384**

(22) Filed: **Dec. 6, 2022**

(65) **Prior Publication Data**

US 2023/0175205 A1 Jun. 8, 2023

**Related U.S. Application Data**

(60) Provisional application No. 63/287,355, filed on Dec. 8, 2021.

(51) **Int. Cl.**

**D21D 1/34** (2006.01)  
**D21B 1/14** (2006.01)  
**D21D 1/40** (2006.01)  
**D21H 17/67** (2006.01)

(52) **U.S. Cl.**

CPC ..... **D21D 1/34** (2013.01); **D21B 1/14** (2013.01); **D21D 1/40** (2013.01); **D21H 17/67** (2013.01)

(58) **Field of Classification Search**  
CPC ..... D21C 1/04; D21C 5/00; D21C 5/005;  
D21H 17/67; D21D 1/34; D21D 1/40;  
D21B 1/14

See application file for complete search history.

(56) **References Cited**

**U.S. PATENT DOCUMENTS**

|                  |         |                               |
|------------------|---------|-------------------------------|
| 4,978,364 A      | 12/1990 | Walker                        |
| 6,066,494 A      | 5/2000  | Hsieh                         |
| 7,771,565 B2     | 8/2010  | Kirov                         |
| 11,421,257 B2    | 8/2022  | Farrell et al.                |
| 2009/0044345 A1* | 2/2009  | Schlingloff ..... A61L 12/128 |
| 2016/0160253 A1  | 6/2016  | Larsen                        |

8/111

(Continued)

**FOREIGN PATENT DOCUMENTS**

|                    |         |
|--------------------|---------|
| WO 2021003077 A1   | 1/2021  |
| WO 2021226094 A1 * | 11/2021 |
| WO 2023107947 A1   | 6/2023  |

**OTHER PUBLICATIONS**

International Search Report for PCT/US2022/081020, mailed Jun. 15, 2023.

(Continued)

*Primary Examiner* — Jacob T Minskey

*Assistant Examiner* — Elisa H Vera

(74) *Attorney, Agent, or Firm* — McBee Moore & Vanik IP, LLC

(57) **ABSTRACT**

Disclosed is mechanical and decolorization pretreatment of cotton-containing textiles, such as “trash” feedstock in terms of end-of-life-cotton textiles, that may be used to produce sugar without the use of harsh pretreatments conditions.

**28 Claims, 4 Drawing Sheets**



(56)

**References Cited****U.S. PATENT DOCUMENTS**

2016/0201102 A1 7/2016 Zhu et al.  
2021/0269969 A1\* 9/2021 Breliid ..... B29B 17/0412

**OTHER PUBLICATIONS**

- Written Opinion for PCT/US2022/081020, mailed Jun. 15, 2023.
- Wyman et al., "Simultaneous Saccharification and Fermentation of Several Lignocellulosic Feedstocks to Fuel Ethanol," *Biomass and Bioenergy*, 1992, 3(5): 301-307.
- "Laboratory beating of pulp (PFI mill method)," approved by the Pulp Properties Committee of the Process and Product Quality Division, TAPPI, 2000, pp. 1-6.
- "Textiles: Material-Specific Data," retrieved from <<https://epa.gov/facts-and-figures-about-materials-waste-and-recycling/textiles-material-specific-data>> on Oct. 7, 2021, pp. 1-5.
- Beall, "Why are clothes so hard to recycle," Jul. 12, 2020, British Broadcasting Corporation website, pp. 1-10.
- Li et al., "Biodegradability study on cotton and polyester fabrics," *J. Eng. Fiber. Fabr.*, vol. 5, No. 4, pp. 42-53, 2010.
- Singh and Satapathy, "Conversion of Lignocellulosic Biomass to Bioethanol: An Overview with a Focus on Pretreatment," *Int. J. Eng. Technol.*, vol. 15, pp. 17-43, 2018.
- Rojas (ed.), "Cellulose Chemistry and Properties : Fibers, Nanocelluloses and Advanced Materials," (book), Springer, New York, 2016, ISSN: 0065-3195.
- Hamawand et al., "Bioenergy from Cotton Industry Wastes: A review and potential," *Renew. Sustain. Energy Rev.*, vol. 66, pp. 435-448, 2016.
- Johnson et al. "Supply Chain of Waste Cotton Recycling and Reuse : A Review," *AATCC Journal of Research*, 2020, 7(1):19-31, abstract only.
- Alvira et al. "Pretreatment technologies for an efficient bioethanol production process based on enzymatic hydrolysis: A review," *Bioresour. Technol.*, 2010, 101(13): 4851-4861.
- Abatti De Assis et al., "Risk management consideration in the bioeconomy," *Biofuels, Bioprod. Biorefining*, 2017, 11: 549-566, abstract only.
- Chandra et al., "Substrate pretreatment: The key to effective enzymatic hydrolysis of lignocellulosics?," *Adv. Biochem. Eng. Biotechnol.*, 2007, 108: 67-93.
- Bajpai, "Pretreatment of Lignocellulosic Biomass," Springer, Singapore, 2016, Chapter 4, pp. 17-70.
- Heinze et al, *Cellulose Chemistry and Properties : Fibers , Nanocelluloses and Advanced Materials*, vol. 271. Springer International Publishing, 2016 (book): 1-52.
- Hendricks et al., "Pretreatments to enhance the digestibility of lignocellulosic biomass," *Bioresour. Technol.*, 100(1): 10-18, Jan. 2009.
- Corbett et al., "Fiber fractionation to understand the effect of mechanical refining on fiber structure and resulting enzymatic digestibility of biomass," *Biotechnol. Bioeng.*, 2020, 117: 924-932.
- De Assis et al., "Toward an understanding of the increase in enzymatic hydrolysis by mechanical refining," 2018, *Biotechnol. Biofuels*, vol. 11, pp. 1-11.
- Gharehkani et al., "Basic effects of pulp refining on fiber properties—A review," 2015, *Carbohydr. Polym.*, El Sevier, 115: pp. 1-5.
- Buschle-Diller & Traore, "Influence of direct and reactive dyes on the enzymatic hydrolysis of cotton," *Textile Research Journal*, 1998, 68(3): 185-192.
- Chakraborty et al., Modeling energy consumption for the generation of microfibres from bleached kraft pulp fibres in a PFI mill, *BioResources*, 2007, pp. 210-222, vol. 2-2.

\* cited by examiner



FIG. 1



FIG. 2



FIG. 3



FIG. 4



FIG. 5



FIG. 6

## PRETREATMENT METHODS FOR COTTON TEXTILE WASTE FABRIC

### CROSS-REFERENCE TO RELATED APPLICATIONS

This application claims priority to U.S. Application No. 63/287,355, filed 8 Dec. 2021, the disclosure of which is herein incorporated by reference in its entirety.

### FIELD OF THE INVENTION

This disclosure relates to a process for producing sugar from cotton-containing textiles.

### BACKGROUND OF THE INVENTION

The Environmental Protection Agency (EPA) estimates that the United States in 2018 combusted 3.2 million tons of textile waste and landfills receives 11.3 million tones of textile waste. EPA “Textiles: Material-Specific Data” EPA Website (2021). If discarded in a landfill, these textiles contribute to the emission of greenhouse gases (e.g., methane) as they degrade. Further, the degradation process for synthetic fibers (e.g., polyesters) can take hundreds of years. If the textile waste is incinerated, toxic gases can be released, especially from more complex textile blends. BBC Website “Why Clothes are so hard to recycle.” (Jul. 12, 2020).

Textile waste represents 3% of the global waste market share. Hamawand et al., “Bioenergy from Cotton Industry Wastes: A review and potential,” *Renew. Sustain. Energy Rev.*, vol. 66, pp. 435-448, 2016; Johnson et al. “Supply Chain of Waste Cotton Recycling and Reuse: A Review,” 2020. It is the 10th most generated waste after food, paper, plastic, and glass derived waste. Degradation time for cotton fabric is approximately 50-77% in 90 days. Li, Frey, and Browning, “Biodegradability study on cotton and polyester fabrics,” *J. Eng. Fiber. Fabr.*, vol. 5, no. 4, pp. 42-53, 2010.

There exists a need in the art for methods for processing textile waste into sugar and other value-added products.

### SUMMARY OF THE INVENTION

In an embodiment, a method of pretreating cotton-containing textile material may comprise refining the cotton-containing textile material in a PFI mill for between about 2,000 and 20,000 revolutions.

In an embodiment, a method of pretreating cotton-containing textile material may comprise decolorizing the cotton-containing textile material and refining the cotton-containing textile material in a PFI mill for between about 2,000 and 20,000 revolutions.

The method may further comprise additional pretreatment. The additional pretreatment may comprise mechanical pretreatment, chemical, enzymatic pretreatment, or a combination thereof. The method may further comprise shredding the cotton-containing textile material, cutting the cotton-containing textile material, and milling the cotton-containing textile material prior to refining the cotton-containing textile material in PFI mill.

In an embodiment, a method of processing cotton-containing textile material may comprise (a) shredding the cotton-containing textile material; (b) cutting the cotton-containing textile material; (c) milling the cotton-containing textile material; (d) refining the cotton-containing textile material in a PFI mill for between about 2,000 and 20,000

revolutions; and (e) subjecting the pretreated cotton-containing textile material to hydrolysis to produce a hydrolysate. In an embodiment, the method may further comprise decolorizing the cotton-containing textile material after cutting and milling, but before refining.

In an embodiment, method of processing cotton-containing textile material may comprise (a) shredding the cotton-containing textile material; (b) cutting the cotton-containing textile material; (c) milling the cotton-containing textile material; (d) decolorizing the cotton-containing textile material; (e) refining the cotton-containing textile material in a PFI mill for between about 2,000 and 20,000 revolutions; and (f) subjecting the pretreated cotton-containing textile material to hydrolysis to produce a hydrolysate.

15 In an embodiment, the decolorizing step may comprise bleaching. The bleaching may comprise treatment with ozone, sodium hypochlorite, hydrogen peroxide, a Fenton’s reagent, or a combination thereof. The hydrogen peroxide may be in a range from about 1.0% to about 8.0% (w/w). The hydrogen peroxide may be in the range of about 2.0% to 6.0%, 4.0% and 8.0%, 5.0% and 7% (w/w).

20 In an embodiment, the bleaching may further comprise treatment with sodium hydroxide. The sodium hydroxide may be in a range from 1.0% to about 6.0%, or optionally in a range from 2.0% to 4.0% (w/w). The sodium hydroxide may be in the range of from about 2.0% to 4.0%, 3.0% to 5.0%, 4.0% to 6.0%, or 1.0% to 5.0% (w/w). The sodium hydroxide may be in an amount of about 1.0%, 2.0%, 3.0%, 4.0%, 5.0%, or 6.0% (w/w).

25 In an embodiment, the method may further comprise adding Cu<sup>2+</sup>. The Cu<sup>2+</sup> may be added in the range of 100 ppm to 250 ppm. The range may be from about 120 ppm to 170 ppm. The amount may be about 100 ppm, 101 ppm, 102 ppm, 103 ppm, 104 ppm, 105 ppm, 106 ppm, 107 ppm, 108 ppm, 109 ppm, 110 ppm, 111 ppm, 112 ppm, 113 ppm, 114 ppm, 115 ppm, 116 ppm, 117 ppm, 118 ppm, 119 ppm, 120 ppm, 121 ppm, 122 ppm, 123 ppm, 124 ppm, 125 ppm, 126 ppm, 127 ppm, 128 ppm, 129 ppm, 130 ppm, 131 ppm, 132 ppm, 133 ppm, 134 ppm, 135 ppm, 136 ppm, 137 ppm, 138 ppm, 139 ppm, 140 ppm, 141 ppm, 142 ppm, 143 ppm, 144 ppm, 145 ppm, 146 ppm, 147 ppm, 148 ppm, 149 ppm, 150 ppm, 151 ppm, 152 ppm, 153 ppm, 154 ppm, 155 ppm, 156 ppm, 157 ppm, 158 ppm, 159 ppm, 160 ppm, 161 ppm, 162 ppm, 163 ppm, 164 ppm, 165 ppm, 166 ppm, 167 ppm, 168 ppm, 169 ppm, 170 ppm, 171 ppm, 172 ppm, 173 ppm, 174 ppm, 175 ppm, 176 ppm, 177 ppm, 178 ppm, 179 ppm, 180 ppm, 181 ppm, 182 ppm, 183 ppm, 184 ppm, 185 ppm, 186 ppm, 187 ppm, 188 ppm, 189 ppm, 190 ppm, 191 ppm, 192 ppm, 193 ppm, 194 ppm, 195 ppm, 196 ppm, 197 ppm, 198 ppm, 199 ppm, 200 ppm, 201 ppm, 202 ppm, 203 ppm, 204 ppm, 205 ppm, 206 ppm, 207 ppm, 208 ppm, 209 ppm, 210 ppm, 215 ppm, 220 ppm, 225, 230 ppm, 235 ppm, 240 ppm, 245 ppm, or 250 ppm.

30 In an embodiment, the method may further comprise adding Fe<sup>2+</sup>. The Fe<sup>2+</sup> may be added in the range of 100 ppm to 250 ppm. The range may be from about 120 ppm to 170 ppm. The amount may be about 100 ppm, 101 ppm, 102 ppm, 103 ppm, 104 ppm, 105 ppm, 106 ppm, 107 ppm, 108 ppm, 109 ppm, 110 ppm, 111 ppm, 112 ppm, 113 ppm, 114 ppm, 115 ppm, 116 ppm, 117 ppm, 118 ppm, 119 ppm, 120 ppm, 121 ppm, 122 ppm, 123 ppm, 124 ppm, 125 ppm, 126 ppm, 127 ppm, 128 ppm, 129 ppm, 130 ppm, 131 ppm, 132 ppm, 133 ppm, 134 ppm, 135 ppm, 136 ppm, 137 ppm, 138 ppm, 139 ppm, 140 ppm, 141 ppm, 142 ppm, 143 ppm, 144 ppm, 145 ppm, 146 ppm, 147 ppm, 148 ppm, 149 ppm, 150 ppm, 151 ppm, 152 ppm, 153 ppm, 154 ppm, 155 ppm, 156 ppm, 157 ppm, 158 ppm, 159 ppm, 160 ppm, 161 ppm, 162

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400

ppm, 163 ppm, 164 ppm, 165 ppm, 166 ppm, 167 ppm, 168 ppm, 169 ppm, 170 ppm, 171 ppm, 172 ppm, 173 ppm, 174 ppm, 175 ppm, 176 ppm, 177 ppm, 178 ppm, 179 ppm, 180 ppm, 181 ppm, 182 ppm, 183 ppm, 184 ppm, 185 ppm, 186 ppm, 187 ppm, 188 ppm, 189 ppm, 190 ppm, 191 ppm, 192 ppm, 193 ppm, 194 ppm, 195 ppm, 196 ppm, 197 ppm, 198 ppm, 199 ppm, 200 ppm, 201 ppm, 202 ppm, 203 ppm, 204 ppm, 205 ppm, 206 ppm, 207 ppm, 208 ppm, 209 ppm, 210 ppm, 215 ppm, 220 ppm, 225, 230 ppm, 235 ppm, 240 ppm, 245 ppm, or 250 ppm.

In an embodiment, the bleaching may be conducted at a temperature range of 60° C. to 120° C. The temperature may be in a range of about 80° C. to 100° C. The bleaching may be conducted at a temperature of between about 100° C. to 110° C., 90° C. to 100° C., 90° C. to 110° C., or 95° C. to 120° C. The temperature may be about 80° C., 81° C., 82° C., 83° C., 84° C., 85° C., 86° C., 87° C., 88° C., 89° C., 90° C., 91° C., 92° C., 93° C., 94° C., 95° C., 96° C., 97° C., 98° C., 99° C., 100° C., 101° C., 102° C., 103° C., 104° C., 105° C., 106° C., 107° C., 108° C., 109° C., 110° C., 111° C., 112° C., 113° C., 114° C., 115° C., 116° C., 117° C., 118° C., 119° C., or 120° C.

In an embodiment, the bleaching may be conducted for a time in the range of 60 minutes to 120 minutes. The time may be in the range of about 80 minutes to 110 minutes. The time may be in the range of about 80 to 90 minutes, 90 to 100 minutes, 95 to 120 minutes, or 110 to 120 minutes. The time may be about 60, 61, 62, 63, 64, 65, 66, 67, 68, 69, 70, 71, 72, 73, 74, 75, 76, 77, 78, 79, 80, 81, 82, 83, 84, 85, 86, 87, 88, 89, 90, 91, 92, 93, 94, 95, 96, 97, 98, 99, 100, 101, 102, 103, 104, 105, 106, 107, 108, 109, 110, 111, 112, 113, 114, 115, 116, 117, 118, 119, or 120 minutes.

In an embodiment, the decolorization may be performed at a pH between about pH 7 and pH 11. The decolorization may be performed at a pH above pH 10. The decolorization may be performed at about pH 11. The decolorization may be performed at about pH 11.5. The decolorization may be performed at about pH 11.75. The decolorization may be performed at about pH 12.

In an embodiment, a solvent may be added to the cotton-containing textile material prior to refining in a PFI mill. The solvent may be water.

In an embodiment, the method may further comprise enzymatic hydrolysis of the pretreated cotton-containing textile material to produce a hydrolysate.

In an embodiment, the method may further comprise cutting the cotton-containing textile material.

In an embodiment, the method may further comprise milling the cotton-containing textile material.

In an embodiment, the method may further comprise decolorizing the cotton-containing textile material.

In an embodiment, the mechanical pretreatment may comprise shredding, cutting, milling, refining, and combinations thereof.

In an embodiment, the method may further comprise adding a solvent to the cotton-containing textile material during the mechanical pretreatment. The solvent may be water. The solvent may be added before, during, or both before and during refining. The solvent may be added in an amount of between about 1:0.01 and 1:30 mechanically pretreated cotton-containing textile:solvent weight/weight. The amount of solvent added to the cotton-containing textile may be between about 1:0.1 and 1:20, 1:0.1 and 1:10, 1:0.1 and 1:5, or 1:0.1 and 1:0.5 mechanically pretreated cotton-containing textile:solvent weight/weight. The amount of solvent added to the cotton-containing textile may be about 1:0.1, 1:0.2, 1:0.3, 1:0.4, 1:0.5, 1:0.6, 1:0.7, 1:0.8, 1:0.9, or

1:1 mechanically pretreated cotton-containing textile:solvent weight/weight. The amount of solvent added to the cotton-containing textile may be 1:0.2 mechanically pretreated cotton-containing textile:solvent weight/weight.

In an embodiment, the mechanical pretreatment may be conducted at a temperature between about 0° C. and 50° C. The mechanical pretreatment may be conducted at a temperature between about 10° C. and 40° C. The mechanical pretreatment may be conducted at a temperature of about 10° C., 11° C., 12° C., 13° C., 14° C., 15° C., 16° C., 17° C., 18° C., 19° C., 20° C., 21° C., 22° C., 23° C., 24° C., 25° C., 26° C., 27° C., 28° C., 29° C., 30° C., 31° C., 32° C., 33° C., 34° C., 35° C., 36° C., 37° C., 38° C., 39° C., or 40° C. The mechanical pretreatment may be conducted at a temperature of about 25° C.

In an embodiment, the mechanically pretreated cotton-containing textile material may comprise between about 1% and 50% fines by weight. The mechanically pretreated cotton-containing textile material may comprise between about 1% and 20% fines by weight, 25% and 50% fines by weight, 10% and 30% fines by weight, 30% and 50% fines by weight, or 15% and 35% fines by weight. The mechanically pretreated cotton-containing textile material may comprise between about 1%, 2%, 3%, 4%, 5%, 6%, 7%, 8%, 9%, 10%, 11%, 12%, 13%, 14%, 15%, 16%, 17%, 18%, 19%, 20%, 21%, 22%, 23%, 24%, 25%, 26%, 27%, 28%, 29%, 30%, 31%, 32%, 33%, 34%, 35%, 36%, 37%, 38%, 39%, 40%, 41%, 42%, 43%, 44%, 45%, 46%, 47%, 48%, 49%, or 50% fines by weight.

In an embodiment, the fiber length LWL (mm) of the mechanically pretreated cotton-containing textile material may be between about 0.1 mm and 2.00 mm. The fiber length LWL (mm) of the mechanically pretreated cotton-containing textile material may be between about 0.1 mm, 0.2 mm, 0.3 mm, 0.4 mm, 0.5 mm, 0.6 mm, 0.7 mm, 0.8 mm, 0.9 mm, 1.0 mm, 1.1 mm, 1.2 mm, 1.3 mm, 1.4 mm, 1.5 mm, 1.6 mm, 1.7 mm, 1.8 mm, 1.9 mm, or 2.00 mm.

In an embodiment, the level of refining may be between about 2,000 and 20,000 PFI revs. The level of refining may be between about 2,000 and 10,000 PFI revs; 5,000 and 15,000 PFI revs; 5,000 and 20,000 PFI revs; or 10,000 and 20,000 PFI revs. The level of refining may be at about 2,000; 3,000; 4,000, 5,000; 6,000; 7,000; 8,000; 9,000; 10,000; 11,000; 12,000; 13,000; 14,000, 15,000; 16,000; 17,000; 18,000; 19,000; or 20,000 PFI revs.

In an embodiment, the Canadian Standard Freeness (CSF) of mechanically pretreated cotton-containing textile material may be between about 100 and 900 CSF milliliters. The Canadian Standard Freeness (CSF) of mechanically pretreated cotton-containing textile material may be between about 100 and 900 CSF milliliters, 200 and 400 CSF milliliters, 400 and 600 CSF milliliters. The level of refining may be between about 100 and 900 ml CSF milliliters.

In an embodiment, the mechanically pretreated cotton-containing textile may be in the form of a powder. The average particle size of the powder may be between about 0.10 mm and about 2.0 mm.

In an embodiment, a Wiley Mill may be used for the cutting step.

In an embodiment, the mechanical pretreatment may be performed before decolorization of the cotton-textile material.

In an embodiment, the hydrolysis may comprise enzyme hydrolysis comprising the addition of at least one hydrolytic enzyme.

In an embodiment, the enzymatic hydrolysis may comprise the addition combination of a cellulase and  $\beta$ -glucosidase.

In an embodiment, the hydrolysate may comprise a sugar. The sugar may be glucan, xylan, arabinan, mannan, galactan, glucose, sucrose, hexose, or a combination thereof.

In an embodiment, the enzymatic hydrolysis may be conducted at a temperature between about 20° C. and 75° C. The enzymatic hydrolysis may be conducted at a temperature between about 40° C. and 75° C., about 45° C. and 75° C., 50° C. and 75° C., about 55° C. and 75° C., 60° C. and 75° C., or about 65° C. and 75° C. The enzymatic hydrolysis may be conducted at 20° C., 25° C., 30° C., 35° C., 40° C., 45° C., 50° C., 55° C., 60° C., 65° C., 70° C., or 75° C.

In an embodiment, the enzymatic hydrolysis may be conducted at a pH between about pH=4.5 and pH=8.5. The enzymatic hydrolysis may be conducted at a pH of 4.5, 4.6, 4.7, 4.8, 4.9, 5, 5.1, 5.2, 5.3, 5.4, 5.5, 5.6, 5.7, 5.8, 5.9, 6, 6.1, 6.2, 6.3, 6.4, 6.5, 6.6, 6.7, 6.8, 6.9, 7, 7.1, 7.2, 7.3, 7.4, 7.5, 7.6, 7.7, 7.8, 7.9, 8, 8.1, 8.2, 8.3, 8.4, or 8.5.

In an embodiment, the enzymatic hydrolysis may be conducted for between about 1 hour and 300 hours. The enzymatic hydrolysis may be conducted for between about 12 hours and 300 hours, 24 hours and 144 hours, 24 hours and 180 hours, 48 hours and 240 hours, or 24 hours and 96 hours. The enzymatic hydrolysis may be conducted for about 12, 24, 36, 48, 60, 72, 84, 96, 108, 120, 132, 144, 156, 168, 180, 192, 204, 216, 228, 240, 252, 264, 276, 288, or 300 hours. The enzymatic hydrolysis may be conducted for about 24, 36, 48, 60, 72, 84, 96, 108, 120, 132, 144, 156, 168, 180, or 192 hours.

In an embodiment, the amount of enzyme used in the enzymatic hydrolysis may be between about 1 FPU and 50 FPU/g cotton. The amount of enzyme used in the enzymatic hydrolysis may be about 1, 2, 3, 4, 5, 6, 7, 8, 9, 10, 11, 12, 13, 14, 15, 16, 17, 18, 19, 20, 21, 22, 23, 24, 25, 26, 27, 28, 29, 30, 31, 32, 33, 34, 35, 36, 37, 38, 39, 40, 41, 42, 43, 44, 45, 46, 47, 48, 49, or 50 FPU.

In an embodiment, the amount of enzyme used in the enzymatic hydrolysis may be between about 0.01% and 10% enzyme/cotton (w/w), optionally between about 0.02% to 0.05% enzyme/cotton (w/w).

In an embodiment, the enzymatic hydrolysis efficiency may be at least 50%, at least 60%, at least 65%, or at least 70%.

In an embodiment, the enzymatic hydrolysis may further comprise the addition of an acid, base, or both for pH control. The acid may be acetic acid, citric acid, or a combination thereof.

In an embodiment, the method may further comprise filtering the hydrolysis product to produce a permeate and retentate, wherein the permeate may comprise the hydrolysate and the retentate may comprise the residue.

In an embodiment, the method may further comprise subjecting the hydrolysate to fermentation, oxidation, reduction, or hydrogenation to produce an end product.

In an embodiment, the method may further comprise subjecting the hydrolysate to fermentation.

In an embodiment, the end products produced by fermentation comprise alcohols, sugar alcohols, acids, fatty acids, gases, amino acids, chemicals, and mixtures thereof. The sugar alcohols may comprise sorbitol, xylitol, ethylene glycol, glycerol, erythritol, threitol, arabitol, ribitol, mannitol, galactitol, fucitol, iditol, inositol, volemitol, isomalt, lactitol, and mixtures thereof. The alcohols may comprise ethanol, butanol, methanol, propanol, and mixtures thereof. The acids may comprise 2,5-furandicarboxylic acid, itaconic

acid, levulinic acid, succinic acid, lactic acid, malic acid, citric acid, acrylic acid, fumaric acid, hydroxypropionic acid, acrylic acid, and mixtures thereof. The chemicals may comprise glycerol, 3-hydropropanoic acid, 2,5-dimethylfuran (DMF), 5-hydroxymethyl furfural (HMF), furfural, aldehydes, amines, terephthalic acid, hexamethylenediamine, isoprene, polyhydroxyalkanoates, 1,3-propanediol, or mixtures thereof. The gases may comprise methane, ethane, CO, CO<sub>2</sub>, and H<sub>2</sub>, or mixtures thereof.

10 In an embodiment, the enzymatic hydrolysis and fermentation may occur simultaneously.

In an embodiment, the enzymatic hydrolysis and fermentation may be conducted separately.

In an embodiment, the method may not comprise a 15 pretreatment step that requires neutralization from use of an acid or base, recovery of any solvent, or rinsing steps necessitated from a pretreatment that requires components to be removed before hydrolysis and/or fermentation.

In an embodiment, a method may not comprise a step that 20 requires the use of an acid.

In an embodiment, mechanical pretreatment may be substantially free of the use of chemicals.

In an embodiment, a system for the production of sugars 25 from a cotton-containing textile material may comprise a shredding means, cutting means, milling means, refining means, and an enzymatic hydrolysis reactor all mechanically coupled together in series.

#### BRIEF DESCRIPTION OF THE FIGURES

30 FIG. 1 depicts the cotton fibers after mechanical refining, (A) Shredding, (B) Wiley Mill; (C) PFI 2500 rev; (D) PFI 5,000 rev; (E) PFI 10,000 rev; and (F) PFI 20,000 rev. Included below are the fiber length LWL (mm) and the percentage of fiber fines weighted.

35 FIG. 2 depicts the enzymatic hydrolysis of cotton textile waste (50° C., pH=5.2, 6 FPU) for 96 hours versus 192 hours as compared to no refining. Cotton conversion (%) is shown on the left X-axis and percentage of fines on the right X axis. 40 The level of refining with PFI as measured by (rev). Finally, the energy consumed per ton of cotton equivalent to each level of the refining is shown at the bottom. For example, 900 KWh would be needed to refine 1 ton of cotton at 5,000 PFI revs.

45 FIG. 3 depicts the cotton conversion (%) as a function of refining as measured by PFI revolutions. The enzymatic hydrolysis was carried out at 50° C., pH=5.2, 5 FPU for 48, 72, 96, or 192 hours. The efficiency of the cotton conversion as measured by percentage (%) based on initial mass of cotton increased with increased PFI revolutions.

50 FIG. 4 depicts the cotton conversion (%) as a function of refining as measured by hours of reaction time. The enzymatic hydrolysis was carried out at 50° C., pH=5.2, 5 FPU. The efficiency of the cotton conversion as measured by percentage (%) based on initial mass of cotton increased with increased reaction time.

55 FIG. 5 depicts the cotton conversion (%) as a function of refining as measured by PFI revolutions. The enzymatic hydrolysis was carried out at 50° C., pH=5.2, 5 FPU (4.4% g enzyme/g OD cotton) or 6 FPU (5.1% g enzyme/g OD cotton) for 96 hours. The experiments were run in duplicate. The efficiency of the cotton conversion as measured by percentage (%) based on initial mass of cotton increased with increased PFI revolutions, with 6 FPU producing about 6% more cotton conversion than 5 FPU.

60 FIG. 6 depicts the cotton conversion (%) as a function of refining as measured by PFI revolutions. The enzymatic

hydrolysis was carried out at 50° C., pH=5.2, 5 FPU (4.4% g enzyme/g OD cotton) or 6 FPU (5.1% g enzyme/g OD cotton) for 192 hours. The experiments were run in duplicate. The efficiency of the cotton conversion as measured by percentage (%) based on initial mass of cotton increased with increased PFI revolutions. Both reactions run at 5 FPU or 6 FPU produced reached 92% cotton conversion.

#### DETAILED DESCRIPTION OF THE INVENTION

The processes of the present disclosure obtain high sugar yields from cotton-containing textiles comprising mechanical pretreatment in a PFI mill to refine the cotton-containing textiles.

Cotton textile waste from fabric has been found to be a promising biomass for the production of bioethanol as a renewable fuel source. According to this disclosure, cotton textiles, such as “trash” feedstock in terms of end-of-life-cotton textiles, may be used to produce sugar without the same kinds of harsh pretreatments used for other biomasses, such as corn, grass sources, or wood. It is known that cotton has higher crystallinity (than such other biomasses), which makes obtaining very high yields of sugar from cotton very challenging. The inventors surprisingly discovered that, despite having higher crystallinity, cotton in the form of cotton textiles can be used to obtain high yields of sugar using the methods described herein.

The methods described herein provide for more efficient pre-treatment of cotton textile containing waste, wherein the cotton fibers produced by the pretreatment have shorter fiber length, a greater percentage of fines by weight, and more disrupted cellulosic fibers. This leads to an unexpected improvement in the processing of the pretreated cotton textile containing waste into sugars, and downstream, into chemicals.

#### Definitions

In the following, some definitions of terms frequently used in this specification to characterize the invention are provided. These terms will, in each instance of its use, in the remainder of the specification have the respectively defined meaning and preferred meanings.

As used in this specification and the appended claims, the singular forms “a”, “an”, and “the” include plural referents, unless the content clearly dictates otherwise.

“Fines,” as used herein, refers broadly to fibers that are small enough to pass through a mesh screen that has a perforation diameter of 76  $\mu\text{m}$  and also contributes to the final properties of a product. Fischer et al. “Pulp Fines-Characterization, Sheet Formation, and Comparison to Microfibrillated Cellulose” *Polymers* 9 (366): 2017

“Fiber length LWL,” as used herein, refers broadly to pulp term related to average length weighted length. “The Application of Fiber Quality Analysis (FQA) and Cellulose Accessibility Measurements To Better Elucidate the Impact of Fiber Curls and Kinks on the Enzymatic Hydrolysis of Fibers” Richard P. Chandra, Jie Wu, and Jack N. Saddler *ACS Sustainable Chemistry & Engineering* 2019 7 (9), 8827-8833.

Filter Paper Cellulase Activity (FPU),” as used herein, refers broadly to the amount of enzyme which produces 2.0 mg of released sugar from 50 mg of filter paper (Whatman No. 1) within 1 hour.

“Cotton-containing Textiles,” as used herein, refers broadly to any textile containing cotton fibers.

“Textile cotton” or “recycled textile cotton,” as used herein, refers broadly to a collected raw material (e.g., clothing at the end of its service life, scraps of fabrics from the garment industry, lint) that is a waste and the cotton component by nature is composed of more than 90% cellulose (which can be converted into sugar).

“Canadian Standard Freeness (CSF)” as used herein, refers broadly to mechanically pretreated cotton-containing textile material. Canadian Standard freeness (CSF) is directly related to the intensity of mechanical refining. It provides a measure of the rate at which a dilute suspension of pulp (e.g., cotton fibers) is dewatered under specified conditions. The dewatering ratio change proportionally inverse to the level of refining.

#### Textile Waste and Processing

Current methods to transform cellulosic textile waste into bio-based building blocks are few, and they are based on acid or alkaline chemical usage with yields between 40 and 90% under very aggressive conditions (high chemical charge). These proposed pathways are capital investment intensive, with high conversion cost, mainly related to the high chemical use, and with subsequent issues related to chemical recovery, resulting thus in high carbon and environmental footprint. Alvira et al. “Pretreatment technologies for an efficient bioethanol production process based on enzymatic hydrolysis: A review,” *Bioresour. Technol.* (2010) 101 (13): 4851-4861. The development of a technology capable of converting recycled/used garments into bio-based building blocks that are sustainable and industrially feasible could represent an important contribution to the cotton and recycled waste business. Abbati De Assis et al., “Risk management consideration in the bioeconomy,” *Biofuels, Bioprod. Biorefining* (2017) 11:549-566.

Because of the aggressive pretreatment required to obtain sugar from cotton biomass (e.g., plant, stalk, gin trash), cotton has not been considered as a high value biomass feedstock. Additionally, cotton typically has a higher degree of crystallinity than other sources of cellulose that makes bioconversion even more challenging. O. J. Rojas, *Cellulose Chemistry and Properties: Fibers, Nanocelluloses and Advanced Materials*. 2016. However, cotton in the form of textiles is 90%+ pure cellulose (and subsequently glucose) that has already been processed and, at the end of life of the consumer good, is essentially a free feedstock for bioprocessing. If end-of-life cotton garments are utilized instead of biomass grown for use as a feedstock, an environmental benefit is obtained, in addition to economic benefits.

For production of sugar from cotton textiles, the use of exotic solvents, high levels of acids, or high levels of caustic at low temperatures have been barriers to commercialization. These processes are not commercially viable due to cost and additional materials needed to neutralize high levels of acid or caustic, recovering and recycling solvents along with the costs of the solvents, and for caustic, maintaining a temperature near freezing. In addition to neutralizing the acid or caustic, the neutralized component needs further to be rinsed.

Cellulose has been used for as a feedstock for ethanol and glucose production, via enzymatic hydrolysis and fermentation. Different pretreatment methods have been used to hinder the effect of hemicellulose and lignin on enzymatic hydrolysis, and therefore to make cellulose available to enzymes. In the case of cotton textile waste, cellulose is further available for enzymatic hydrolysis due to the very low content of hemicellulose and lignin residues. Therefore other issues must be addressed to increase the yield of

glucose and ethanol production, e.g., cellulose crystallinity, degree of polymerization and fiber size, and porosity.

The enzymatic hydrolysis process has been used to degrade cellulose to glucose. However, in cotton textile waste, conversion of cellulose to glucose is slow unless fibers are subjected to some form of pretreatment, due to the high degree of crystallinity and small pore size, which generates difficulties in the availability of cellulose molecules to react with enzymes. Chandra et al., "Substrate pretreatment: The key to effective enzymatic hydrolysis of lignocellulosics?", *Adv. Biochem. Eng. Biotechnol.* (2007) 108:67-93. The availability of cellulose for enzymatic hydrolysis of cotton waste materials is a factor in increasing the yield of glucose and ethanol production. Among the physicochemical properties that influence the yield of glucose in enzymatic hydrolysis of cellulose are specific surface area and cellulose crystallinity and degree of polymerization.

The methods described herein efficiently disrupt the cellulose structure and permit accessibility of enzymes during hydrolysis (saccharification) of cellulose to produce sugars (e.g., glucose). No harsh pretreatment is required. The inventors found that processing unrefined cotton-containing textiles resulted in low cellulose conversion. The mechanical refining methods described herein resulted in the delamination and fibrillation of the cotton fiber in a PFI mill at 5,000 rev resulted in greater cellulose conversion and did not require the use of any chemicals. For example, using a PFI mill at 10,000 rev resulted in 84% conversion using (enzyme 5 FPU) and 90% conversion (enzyme 6 FPU). [unit of filter paper cellulase activity].

#### Cotton-Containing Textile

Cellulose is a natural polymer consisting of a linear chain of hundreds to thousands of D-glucose units linked by  $\beta$ -(1,4)-glycosidic bonds. Cellulose content varies according to the biomass source. Among natural fibers containing cellulose, cotton is the biomass that contains the highest percentage of cellulose; its lignin content is almost null, which presents an advantage in processing. Bajpai, "Pretreatment of Lignocellulosic Biomass," Springer, Singapore, (2016) pages 17-70; Singh and K. B. Satapathy, "Conversion of Lignocellulosic Biomass to Bioethanol: An Overview with a Focus on Pretreatment," *Int. J. Eng. Technol.*, vol. 15, pp. 17-43, 2018.

Cotton fibers have a primary wall, a secondary wall, and a central core or lumen. The width of cotton fiber varies between 12 and 20  $\mu\text{m}$  wide. The average degree of polymerization of cotton ranges between 9,000 and 15,000 with an average crystallinity of 73; both of these values are very high in comparison with other lignocellulosic materials like wood pulp (DP=600-1,500 and Crystallinity=35) and viscose rayon (DP=250-450 and Crystallinity=60). O. J. Rojas, *Cellulose Chemistry and Properties: Fibers, Nanocelluloses and Advanced Materials*. 2016.

A typical composition for raw cotton fiber is shown in Table 1. Cotton contains approximately 90% or more cellulose. The non-cellulosic constituents of cotton include proteins, amino acids, and nitrogen-containing compounds, which are mainly in the cuticle and the lumen.

TABLE 1

| Composition of Cotton Fibers |             |           |
|------------------------------|-------------|-----------|
| Constituent                  | Typical (%) | Range (%) |
| Cellulose                    | 95          | 88.0-96.0 |
| Protein                      | 1.3         | 1.1-1.9   |
| Pectic substances            | 0.9         | 0.7-1.2   |

TABLE 1-continued

| Composition of Cotton Fibers |             |           |
|------------------------------|-------------|-----------|
| Constituent                  | Typical (%) | Range (%) |
| Ash                          | 1.2         | 0.7-1.6   |
| Wax                          | 0.6         | 0.4-1.0   |
| Total sugars                 | 0.3         | 0.1-1.0   |
| Organic acids                | 0.8         | 0.5-1.0   |
| Other                        | 1.4         | —         |

Heinze et al, *Cellulose Chemistry and Properties: Fibers, Nanocelluloses and Advanced Materials*, vol. 271. Springer International Publishing, 2016.

15 The cotton-containing textiles processed by the methods described herein may comprise any cotton, cotton-blend garments, including, but not limited to, cotton-polyester blend garments, or mixtures thereof.

#### Mechanical Pretreatment

20 Mechanical pretreatment of the cotton-containing textile may comprise mechanical processes for breaking down the cotton-containing textile including but not limited to, grinding, shredding, cutting, milling, refining, chopping, or garneting. Mechanical pretreatment effectively physically breaks down the textile into smaller components, increases the surface area of the textile components, reduces crystallinity of the textile, or a combination thereof, aiding in subsequent hydrolysis.

25 The equipment commonly used for fiber size reduction includes mills, extruders and fibrillators. The effects of mechanical treatment are mainly achieved due to the high shear forces generated in grinding and milling processes. Fiber fractions of different sizes are accumulated in the largest particles ( $>0.1$ -2 mm), whereas fines increase with the intensity of shear stress in the treatment. Disk milling, which produces more defibrillation and delamination of fibers, has been proven more effective in enhancing cellulose hydrolysis than hammer milling. Grinding, milling, and refining require high energy input; hence they are cost-intensive, which is detrimental to their widescale application. Hendriks and G. Zeeman, "Pretreatments to enhance the digestibility of lignocellulosic biomass," *Bioresour. Technol.*, vol. 100, no. 1, pp. 10-18, January 2009.

30 40 45 50 55 Mechanical refining action consists of three mechanisms that change fiber structure and morphology: cutting (fiber length reduction), shearing (fiber surface fibrillation), and compression (fiber delamination). The mechanisms occur simultaneously but at different relative levels depending on the refining technology.

The length reduction of the fiber occurs due to the cutting action of the refiner plate as two refiner bars pass one another. Fibrillation is generally an external effect and involves the peeling of smaller fiber fragments away from the main fiber mass due to shearing forces. Lastly, delamination is generally an internal effect arising from repeated compression and decompression of fibers as they are squeezed between the bars and grooves of the refiner plates. The level of refining could be between about 5,000 and 20,000 PFI revolutions.

60 65 The impact of mechanical refining on fiber properties could maximize the reactivity of fibers towards enzymatic hydrolysis at lower energy consumption. Microscope image analysis has shown that refining causes separation of cells, surface fibrillation, internal delamination, and generation of fines. These changes collectively can contribute to an

## 11

increase in the accessible surface area and a higher yield of enzymatic hydrolysis of cellulose (an increase in conversion by 10 to 30%).

Mechanical pretreatment may comprise breaking down the cotton-containing textile by shredding, cutting, milling, and then refining the cotton-containing textile material. Exemplary equipment include a ball mill or PFI Mill for milling, a Wiley Mill for cutting, and refiners such as a PFI refiner, a single disk refiner, a double disk refiner and a twin disk refiner.

A preferred mechanical pretreatment method comprises refining in a PFI mill, optionally at between about 5,000 and 20,000 PFI revolutions. The inventors surprisingly discovered that the use of PFI mill to refine the cotton-containing textile produced a pretreated material comprising more fines, smaller, more disrupted cellulose, yields unexpected improvement in results. For example, the cotton-containing textile may be milled in a PFI mill at about 5,000 PFI revolutions (rev), 6,000 rev, 7,000 rev, 8,000 rev, 9,000 rev, 10,000 rev, 11,000 rev, 12,000 rev, 13,000 rev, 14,000 rev, 15,000 rev, 16,000 rev, 17,000 rev, 18,000 rev, 19,000 rev, or 20,000 rev. The cotton-containing textile may be milled in a PFI mill at between about 5,000 PFI revolutions (rev) and 20,000 rev; 5,000 rev and 10,000 rev; 7,500 rev and 15,000 rev; 7,000 rev and 10,000 rev; 10,000 rev and 20,000 rev; 15,000 rev and 20,000 rev; or 17,500 rev and 20,000 rev.

A PFI mill is a machine developed by Papirindustriens Forskningsinstitut—The Norwegian Pulp and Paper Research Institute. It is known in the art as a PFI mill. The PFI mill is a beater featuring a high reproducibility, used for studying the relationship between beating degree of pulp and physical properties. This machine may be used in the preparation stage of paper making. Beating mechanism: a constant load is given to the pulp circulating in between stainless steel roll and cylindrical mill house, which are rotating with a constant difference in circumferential velocity, applying mechanical effects such as shear and compression, thereby performing beating by frictional forces between fibers. The number of rotations is read on the counter. The beating degree is evaluated by the freeness tester. The outcome of the refining is measured, compared and standardized by a property relate to dewatering also known as freeness where a quantitative scale is used, specifically Canadian Standard Freeness. See description number 0027. See also TAPPI (2000) Laboratory Beating of Pulp (PFI Mill Method). T 248 sp-00.

The mechanical pretreatment comprising milling in a PFI mill refines the cotton-containing textile, opening up the cotton fibers to allow better access for the enzymes during hydrolysis. Additionally, the inventors used HPLC analysis to provide a better analysis of the results and better develop the methods.

The mechanical pretreatment may comprises grinding the cotton-containing textile into a powder, optionally using a PFI mill, wherein average particle size of the powder is between about 0.10 mm and about 2.0 mm. The average particle size of the powder may be between about 0.15 mm and about 1.60 mm. The average particle size of the powder may be between about 0.20 mm and about 1.5 mm. The average particle size of the powder may be less than about

## 12

2.0 mm. The average particle size of the powder may be less than about 1.70 mm. For example, the average particle size of the powder may be greater than zero and less than about 0.10 mm, 0.20 mm, 0.30 mm, 0.40 mm, 0.50 mm, 0.60 mm, 0.70 mm, 0.80 mm, 0.90 mm, 1.0 mm, 1.1 mm, 1.2 mm, 1.3 mm, 1.4 mm, 1.5 mm, 1.6 mm, 1.7 mm, 1.8 mm, 1.9 mm, or 2.0 mm.

The inventors found that the mechanical refining action of a PFI mill yielded an unexpected improvement of pretreatment of the cotton-containing textile. The PFI mechanical refining action consists of three mechanisms that significantly change the fiber structure and morphology: cutting (fiber length reduction), shearing (fiber surface fibrillation), and compression (fiber delamination). These mechanisms occur simultaneously but at different relative levels depending on the refining technology. Chen et al. (2013) *Bioresour. Technol.* 147:401-408; Park et al. (2016) *Bioresour. Technol.* 199:59-67. The length reduction of the fiber occurs due to the cutting action of the refiner plate as two refiner bars pass one another. Excessive fiber cutting results in the generation of fines. Fibrillation is generally an external effect and involves peeling smaller fiber fragments away from the main fiber mass due to shearing forces. Lastly, delamination is generally an internal effect arising from repeated compression and decompression of fibers as they are squeezed between the bars and grooves of the refiner plates. Corbett et al. (2020) *Biotechnol. Bioeng.* 117:924-932; De Assis et al. (2018) *Biotechnol. Biofuels* 11. The forces involved in mechanical refining are described, for instance, in Ghareh-kani et al. (2015) *Carbohydr. Polym.* 115:785-803.

The method of the disclosure may be also used for a cotton-containing textile that is already mechanically pretreated. The cotton-containing textile may be ground, shredded, cut, chopped, garneted, or a combination thereof. The cotton-containing textile may be in the form of a powder.

The mechanical pretreatment may further comprise the addition of a solvent to the cotton-containing textile before, during or both before and during pretreatment. the solvent may be water. The amount of solvent added to the cotton-containing textile may be between about 1:0.01 and 1:30 mechanically pretreated cotton-containing textile in a weight/weight ratio. For a PFI mechanical refining process, the amount of solvent added to the cotton-containing textile may be 1:0.2. The amount of solvent added to the cotton-containing textile may be between about 1:0.1 and 1:20, 1:0.1 and 1:10, 1:0.1 and 1:5, or 1:0.1 and 1:0.5. The amount of solvent added to the cotton-containing textile may be about 1:0.1, 1:0.2, 1:0.3; 1:0.4, 1:0.5, 1:0.6, 1:0.7, 1:0.8, 1:0.9, or 1:1. For example, the PFI may be operated at about 5% solids (w/w) and 95% water (w/w). This may be expressed as 1:20 textile:solvent (water).

The temperature of the mechanical pretreatment could be conducted at a temperature between about 0° C. and 100° C.

The inventors surprisingly discovered that they did not need to use any chemicals in the pretreatment of the cotton-containing textile to achieve a very high cotton conversion rate. For example, previous studies used caustic chemicals, high thermal and enzyme expenditure to achieve cotton conversion.

| Substrate                          | Pretreatment Method                                       | Optimum Pretreatment Condition                                      | Enzyme                                               | Yield                           | Polyester Recovery | Author                                                         |
|------------------------------------|-----------------------------------------------------------|---------------------------------------------------------------------|------------------------------------------------------|---------------------------------|--------------------|----------------------------------------------------------------|
| Blue jeans/cotton                  | Shredded and grounded/ NaOH                               | NaOH 12%, 0 C., 96 h                                                | cellulase and b-glucosidase 20 FPU                   | 85.1% 24 h<br>99.1% 96 h<br>90% | —<br>—<br>—        | (Jeihanipour & Taherzadeh, 2009)<br>(Jeihanipour et al., 2010) |
| 50/50 polyesFIG. Ster/cotton       | Shredded and grounded/ N-methyl morpholine-N-oxide (NMMO) | NMMO 85%, 120° C., 2 h                                              | cellulase and b-glucosidase                          | 90%                             | —                  | (Jeihanipour et al., 2010)                                     |
| 40/60 polyester/viscose            | Shredded and grounded/ N-methyl morpholine-N-oxide (NMMO) | NMMO 85%, 120° C., 2 h                                              | cellulase and b-glucosidase                          | 90%                             | —                  | (Jeihanipour et al., 2010)                                     |
| Blue jeans polyester/cotton        | Milled/Phosphoric acid                                    | H <sub>2</sub> PO <sub>3</sub> 85%, 50° C., 7 h                     | cellulase and b-glucosidase<br>7.5 FPU               | 79%                             | 100%               | (Shen et al., 2013)                                            |
| Blue jeans polyester/cotton        | Milled/NaOH/Urea                                          | NaOH 7% Urea 12%, - 20° C., 1 h                                     | cellulase and b-glucosidase                          | 70%                             | 98%                | (Gholamzad et al., 2014)                                       |
| 40/60 polyester/cotton             | Shredded/Pressure/ Sodium Carbonate                       | Na <sub>2</sub> CO <sub>3</sub> 1M, 150° C. 72 h                    | cellulase and b-glucosidase                          | 48%                             | —                  | (Hasanzadeh et al., 2018)                                      |
| Towel (87.7% cotton)               | Steam Explosion                                           | 5.5 Mpa, 271 ° C., 5 min                                            | cellulase and meicelase                              | 42%                             | —                  | (Sasaki et al., 2019)                                          |
| Towel (87.7% cotton)               | Microwave                                                 | H <sub>2</sub> SO <sub>4</sub> 1%, 180° C., 5 min                   | cellulase and meicelase                              | 80.70%                          | —                  | (Sasaki et al., 2019)                                          |
| 60/40 polyester/cotton             | Milled/NaOH/Urea                                          | NaOH 7%, Urea 12%, - 20° C., 6 h                                    | cellulase and b-glucosidase                          | 98%                             | —                  | (X. Li et al., 2019)                                           |
| Medical cotton waste 95% cellulose | thermomechanical + H <sub>2</sub> SO <sub>4</sub>         | 22.5 mM H <sub>2</sub> SO <sub>4</sub> 0.22%, 180-220 C., 20-40 min | cellulase and b-glucosidase<br>CTEC2 20 mg/g biomass | 95.2%                           | —                  | (Giakoumakis et al., 2020)                                     |

In summary, the previous studies relied on high temperatures, large amounts of enzymes, harsh chemicals, and mixtures thereof, to achieve the cotton conversion. In contrast, the methods described herein do not rely on high temperatures, large amounts of enzymes, harsh chemicals, and mixtures thereof, to achieve the cotton conversion. For example, the inventors found that pretreatment with milling in a Wiley Mill followed by refining in a PFI mill at 10,000 revolutions and hydrolysis for 96 hours with either 5 FPU or 6 FPU, yield 84% conversion or 90% conversion, respectfully. (5 FPU=4.4% g enzyme/g cotton and 6 FPU=5.1% g enzyme/g cotton).

For example, the cotton-containing textile may be shredded, cut, milled, and then have water added, and be reined in a PFI mill at between about 5,000 rev and 20,000 rev. Following this, the pretreated cotton-containing textile material is subjected to hydrolysis, using, for example, either 5 FPU or 6 FPU. This yields over 80% conversion of the cotton fibers and the only chemical used is acetic acid or citric acid during the enzymatic hydrolysis steps for pH control. No chemicals are used in the mechanical pretreatment steps. The only solvent used in the mechanical pretreatment step is water.

#### Decolorization

If the cotton-containing textile is a color other than bleached cotton, dyed or printed, or if it has a finish applied to it such as but not limited to a softener, durable press resin, moisture resistant/moisture wicking finish, abrasion resistant finish, antimicrobial finish or flame retardant finish, enzymatic hydrolysis performance is reduced. See Buschle-Diller & Traore (1998). Influence of direct and reactive dyes on the enzymatic hydrolysis of cotton. *Textile Research Journal*, 68 (3), 185-192.

Then the cotton-containing textile may be decolorized to remove dyes or finishes prior to the pretreatment, hydrolysis and/or saccharification. The dyed or finished cotton-containing textile may be subjected to a decolorization process to remove dye and or finished that may interfere with the enzymatic hydrolysis. The inventors surprisingly discovered that the decolorization methods described herein allow for decolorizing without downstream interference with the

enzymes used in hydrolysis and saccharification. For example, decolorization using the methods described herein increased the yield from about 40% to about 80% to 90%. For example, the cotton-containing textile may be decolorized after cutting and milling but before mechanical refining.

The decolorization treatment may comprise removing part of all of the dye or exposing cellulose of the cotton-containing textile to the hydrolyzing materials. The decolorization method may comprise using at least one bleach compound. The bleach compound may be ozone, sodium hypochlorite, hydrogen peroxide, Fenton's reagent, or a combination thereof.

The bleach compound may be hydrogen peroxide. The cotton-containing material may be bleached with hydrogen peroxide in a range from about 1.0% to about 8.0%, optionally in a range from about 2.0% to 6.0%. The hydrogen peroxide may be combined with sodium hydroxide, the sodium hydroxide may be a range from 1.0% to about 6.0%, optionally in a range from 2.0% to 4.0%. The hydrogen and sodium peroxide may be further combined with metals such as Fe<sup>2+</sup> and Cu<sup>2+</sup> in the range of 100 ppm to 250 ppm, optionally in a range from 120 ppm to 170 ppm. In the process, cotton content measured by percentage (%) from the total mixture can be in a range between 1% and 20%.

The decolorization temperature is preferably at a temperature range of 60° C. to 120° C., optionally in a range of 80° C. to 100° C. for time in a range of 60 minutes to 120 minutes, optionally in a range of 80 minutes to 110 minutes in a pH range preferably above 10. For example, the pH range may be between about 9 and 11.

The bleaching compound may be ozone. The ozone pretreatment procedure is disclosed, for example "Kinetics of ozone bleaching of eucalyptus kraft pulp and factors affecting the properties of the bleached pulp," BioRes. 13(1), 425-436. The cotton-containing material is bleached with ozone in a range from about 1.0% to about 20.0% wt, optionally in a range from about 2.0% to 10.0%, at a flow rate in the range from about 0.1 L/min to 20 L/min, optionally in a range from about 0.5 L/min to 10 L/min, or optionally in a range from about 1 L/min to 5 L/min. The ozone flow rate is 0.1 L/min, 0.2 L/min, 0.3 L/min, 0.4

15

L/min, 0.5 L/min, 0.6 L/min, 0.7 L/min, 0.8 L/min, 0.9 L/min, 1 L/min, 1.1 L/min, 1.2 L/min, 1.2 L/min, 1.3 L/min, 1.3 L/min, 1.4 L/min, 1.5 L/min, 1.6 L/min, 1.7 L/min, 1.8 L/min, 1.9 L/min, or 2 L/min. The ozone decolorization time range is in a range of about 1 minute to 60 minutes, optionally in a range of 10 minutes to 30 minutes. In a preferred embodiment, the range is 10 minutes, 12 minutes, 14 minutes, 16 minutes, 18 minutes, 20 minutes, 22 minutes, 24 minutes, 26 minutes, 28 minutes, or 30 minutes. The ozone decolorization in a pH range preferably from 2 to 11, optionally in a range from 3 to 11. The pH may be 3, 7 or 11. In the process, cotton content measured by percentage (%) from the total mixture can range between 1-30%.

In an embodiment, neutralization is carried out after bleaching pretreatment. Neutralization is carried out with Sulfuric acid until pH 7. Then, a washing process with water is performed at room temperature.

#### Acid Pretreatment Cooling Neutralizing

The cotton-containing textile may be, optionally, subjected to an acid pretreatment. The acid pretreatment of step (c) comprises at least one acid. The at least one acid may comprise a weak acid. Examples of weak acids include, but are not limited to, phosphoric acid, citric acid, nitrous acid, lactic acid, benzoic acid, acetic acid, and carbonic acid. In an embodiment, in contrast to strong acids, the weak acids are acids known to not completely dissociate in water. The at least one acid used in the acid pretreatment may comprise phosphoric acid. The concentration of the at least one acid in step (c) is between about 0.01 M and about 0.5 M, optionally between about 0.10 M and about 0.25 M, optionally between about 0.15 M and about 0.20 M.

The at least one acid is added to the powder at a liquor ratio in a range from about 2:1 to about 12:1, optionally in a range from about 4:1 to about 10:1, optionally at about 6:1.

Optionally, step (c) does not comprise addition of a base—i.e., a base is not used in pre-treating the cotton-containing textile. In an embodiment, step (c) does not comprise a pretreatment that requires neutralization from use of a strong acid or base, recovery of any solvent or pretreatment aids, or rinsing steps necessitated from a pretreatment that requires components to be removed before hydrolysis and/or fermentation.

The elevated temperature in step (c) may be in a range from about 115° C. to about 210° C., optionally in a range from about 121° C. to about 137° C., optionally in a range from about 126° C. to about 132° F., optionally at about 130° C. Heating time in step (c) is in a range from about 0.5 to about 5 hours, optionally from about 1 to about 3 hours, optionally about 2 hours. Agitators may optionally be added to the slurry to enhance internal mixing of the slurry. Due to the acid pretreatment, the resulting slurry has a much-lowered viscosity.

Step (c) may comprise cooling the slurry to a temperature in a range from about 48° C. to about 71° C., optionally in a range from about 54° C. to about 65° C., optionally at about 60° C.

Step (e) may comprise of adding at least one base to the slurry from (c) and optionally agitating the slurry. The at least one base may comprise a strong base. Examples of strong bases include, but are not limited to, potassium hydroxide, sodium hydroxide, barium hydroxide, cesium hydroxide, strontium hydroxide, lithium hydroxide, and rubidium hydroxide. The at least one strong base used in step (e) may comprise sodium hydroxide. The concentration of sodium hydroxide may be in a range from about 0.01 M to about 0.5 M. The concentration of sodium hydroxide is sufficient to effectively neutralize the acid previously added.

16

The presence of sodium hydroxide neutralizes phosphoric acid to form sodium phosphate in situ. The slurry is then optionally agitated, optionally between 1 and 120 minutes, and at a temperature in a range from about 48° C. to about 70° C., optionally in a range from about 55° C. to about 65° C., optionally at about 60° C.

Step (e) may comprise adding at least one additional acid to the cotton slurry from step (d) to form a buffer in situ and optionally agitating the slurry. The at least one additional acid used in step (e) may comprise a weak acid. Examples of weak acids include, but are not limited to, phosphoric acid, citric acid, nitrous acid, lactic acid, benzoic acid, acetic acid, and carbonic acid. The weak acids do not completely dissociate in water. The at least one additional acid used in step (e) may comprise citric acid.

The citric acid from step (e) may form a buffer with sodium phosphate from step (d). A citric acid and sodium phosphate buffer is known as a McIlvaine buffer.

The concentration of the at least one acid in step (e) is between about 0.001 M and about 1.0 M, optionally between about 0.010 M and about 0.1 M, optionally between about 0.025 M and about 0.050 M.

#### Saccharification

The pretreated material may be subjected to enzymatic hydrolysis to produce sugars (Saccharification). For example, the pretreated material may be subjected to separate hydrolysis and fermentation (SHF), simultaneous saccharification and fermentation (SSF), or direct microbial conversion (DMC). Wyman et al. (1992) *Biomass and Bioenergy* 3 (5): 301-307.

The sugars produced by the methods described herein include but are not limited to glucan, xylan, arabinan, mannan, galactan, glucose, sucrose, hexose, and combinations thereof. The enzymatic hydrolysis may comprise incubation with a cellulase composition comprising one or more enzymes that hydrolyze a cellulosic material. Cellulase enzymes include but are not limited to endocellulases, exocellulases, cellobiases, oxidative cellulases, and endoglucanases. Other enzymes that may be used include but are not limited to cellobiohydrolases, beta-glycosidases, and combinations thereof. The hydrolysis may further comprise filtering, whereby the hydrolysate is fermented and saccharified to produce ethanol. Alternatively, if filtering does not occur, the hydrolysis may comprise fermenting and saccharifying the slurry from to form ethanol.

The same step may comprise fermenting and saccharifying the hydrolysate, or when the step comprises fermenting and saccharifying the slurry, the prior step may further comprise combining the hydrolysis enzyme with yeast.

The saccharification may comprise adding at least one hydrolytic enzyme, e.g., at least one cellulase, to the pre-treated cotton material to initiate enzymatic hydrolysis of the pretreated cotton material to form a slurry, and optionally agitating the slurry. The enzymatic hydrolysis may be carried out utilizing a cocktail combination of at least one cellulase and  $\beta$ -glucosidase. The enzyme mixtures may comprise hemicellulases, cellulases, endo-glucanases, exoglucanases, and 1-beta-glucosidases. The cellulase may be cellobiohydrolase, endocellulase, exocellulase, cellobiase, endo-beta-1,4-glucanase, beta-1,4-glucanase, or mixtures thereof.

After the hydrolysis cocktail is added to the pretreated cotton material, hydrolysis occurs for between about 24 and about 240 hours, optionally for between about 48 and 216 hours. The hydrolysis may occur for between about 24 and 36 hours, 24 and 144 hours, 24 and 168 hours, or 48 and 216 hours. The hydrolysis may occur for about 1, 2, 3, 4, 5, 6, 7,

8, 9, 10, 11, 12, 13, 14, 15, 16, 17, 18, 19, 20, 21, 22, 23, 24, 25, 26, 27, 28, 29, 30, 31, 32, 33, 34, 35, 36, 37, 38, 39, 40, 41, 42, 43, 44, 45, 46, 47, 48, 49, 50, 51, 52, 53, 54, 55, 56, 57, 58, 59, 60, 61, 62, 63, 64, 65, 66, 67, 68, 69, 70, 71, 72, 73, 74, 75, 76, 77, 78, 79, 80, 81, 82, 83, 84, 85, 86, 87, 88, 89, 90, 91, 92, 93, 94, 95, 96, 97, 98, 99, 100, 101, 102, 103, 104, 105, 106, 107, 108, 109, 110, 111, 112, 113, 114, 115, 116, 117, 118, 119, 120, 121, 122, 123, 124, 125, 126, 127, 128, 129, 130, 131, 132, 133, 134, 135, 136, 137, 138, 139, 140, 141, 142, 143, 144, 145, 146, 147, 148, 149, 150, 151, 152, 153, 154, 155, 156, 157, 158, 159, 160, 161, 162, 163, 164, 165, 166, 167, 168, 169, 170, 171, 172, 173, 174, 175, 176, 177, 178, 179, 180, 181, 182, 183, 184, 185, 186, 187, 188, 189, 190, 191, 192, 193, 194, 195, 196, 197, 198, 199, 200, 201, 202, 203, 204, 205, 206, 207, 208, 209, 210, 211, 212, 213, 214, 215, or 216 hours. The slurry may be agitated.

The temperature during hydrolysis may be in a range from about 20° C. to about 60° C., optionally in a range from about 40° C. to about 55° C., optionally at about 48° C. The temperature during hydrolysis may be about 30° C., about which temperature saccharification and fermentation may occur simultaneously.

The pH of the enzyme solution during hydrolysis can be controlled with an acid or base or both for pH control. The pH during hydrolysis may be chosen by the skilled person and may be between 3.0 and 10.0, optionally in a range from about 4.0 to about 8.0, optionally in a range from about 4.5 to about 6.5. The pH may range up to 3 pH units, or up to 5 pH units. The optimum pH may lie within the limits of pH 3.0 to 9.0, 3.5 to 8.5, 4.0 to 8.0, or 4.0 to 7.5. The pH may be about 4.5, 4.6, 4.7, 4.8, 4.9, 5.0, 5.1, 5.2, 5.3, 5.4, 5.5, 5.6, 5.7, 5.8, 5.9, 6.0, 6.1, 6.2, 6.3, 6.4, or 6.5. For example, the pH may be about 5.2.

The hydrolysis time is 6 hours or more, 10 hours or more, 12 hours or more, 14 hours or more, 16 hours or more, 18 hours or more, 20 hours or more, 30 hours or more, 40 hours or more, 50 hours or more, 60 hours or more, 70 hours or more, 80 hours or more, 90 hours or more, 100 hours or more, 110 hours or more, 120 hours or more, 130 hours or more, 140 hours or more, 150 hours or more, 160 hours or more, 170 hours or more, 180 hours or more, 190 hours or more, or 200 hours or more. The hydrolysis time is 10 to 120 hours.

The activity of the enzyme should be measured between 1 FPU and 540 FPU/g cotton. Developed by the IUPAC, an FPU is a standard way to express enzyme dosage and its ability to convert 50 g of cellulose filter paper into 2.0 mg glucose in 60 minutes. Adney, B. and Baker, J. "Measurements of Cellulase Activities," *NREL Laboratory Technical Report NREL/TP-510-42628*, 2008.

The amount of enzyme to cotton weight ratio ISE between 0.01% and 10.0%.

The hydrolysis efficiency may be determined in a manner known to one of skill in the art. Exemplary analysis methods include Cotton Residue, HPLC, and RIDA® Cube. In an embodiment, hydrolysis efficiency is determined using the RIDA® Cube method. The hydrolysis efficiency is at least about 10%, at least about 20%, at least about 30%, at least about 40%, at least about 50%, at least about 51%, at least about 52%, at least about 53%, at least about 54%, at least about 55%, at least about 56%, at least about 57%, at least about 58%, at least about 59%, at least about 60%, at least about 61%, at least about 62%, at least about 63%, at least about 64%, at least about 65%, at least about 66%, at least about 67%, at least about 68%, at least about 69%, at least about 70%, at least about 71%, at least about 72%, at least about 73%, at least about 74%, at least about 75%, at least

about 76%, at least about 77%, at least about 78%, at least about 79%, or at least about 80%.

The methods described herein may not comprise a pretreatment step that requires neutralization from use of a strong acid or base, recovery of any solvent or pretreatment aids, or rinsing steps necessitated from a pretreatment that requires components to be removed before hydrolysis and/or fermentation.

#### Filtering and Drying

Following the hydrolysis step, the slurry may be filtered to produce a retentate (cotton residue) and a permeate (hydrolysate comprising sugars). This filtering may be done by any conventional means known to those skilled in the art, such as, for example, those described in U.S. Pat. No. 9,540,665, which is herein incorporated by reference. The cotton residue is then dried, for example in an oven, and optionally weighed after drying. The cotton residue is dried in an oven at a temperature in a range from about 48° C. to about 82° C., optionally in a range from about 60° C. to about 76° C., optionally at about 70° C. The drying time may optionally be at least about 2 hours, optionally in a range from about 4 to about 48 hours, optionally in a range from about 10 to about 24 hours, optionally at least about 16 hours.

After drying, a conversion rate (or hydrolysis efficiency) may be calculated. For example, after drying, the cotton residue may be weighed at time=0 minutes and time≥15 minutes. The conversion rate is then calculated based on the amount of cotton added and the weight of residue at time≥15 minutes. In an embodiment, HPLC and RIDA® Cube are analysis methods that may be used to measure glucose concentration of the solution to calculate the hydrolysis efficiency.

In another embodiment, cellulose conversion efficiency is calculated. The amount of cellulose in a garment is predetermined by an acid burnout. An HPLC is then performed to quantify the glucose in the hydrolyzed sample. The determined glucose is compared to the theoretical amount of glucose in the sample based on the following formula:

$$\text{Cellulose conversion(%) = } \% \text{ cellulose converted into glucose} / \% \text{ initial cellulose in the system} * 100 \quad (1)$$

$$\text{Cellulose conversion(%) = } (\% \text{ glucose in HPLC}) * 0.9 / [(\% \text{ cotton in initial system}) * \text{cellulose content in cotton}] * 100 \quad (2)$$

Where:

$$\% \text{ cellulose converted into glucose} = (\% \text{ glucose in HPLC}) * 0.9 \quad (3)$$

$$\% \text{ initial cellulose in the system} = (\% \text{ cotton in the initial system}) * \text{cellulose content in cotton} \quad (4)^*$$

(4)\*Cellulose content in cotton is determined through compositional analysis using TAPPI and NREL standard method Conversion of Sugars to End Products

The sugars produced by the methods described herein may further undergo biochemical treatment (e.g., fermentation) to produce end products. For example, the sugars produced by the methods described herein may be contacted with a microorganism in a fermentation process to produce end products. The sugars produced by the methods described herein may be contacted with an enzyme, or a mixture of enzymes, in a fermentation process to produce end products. The end products produced by fermentation, may include but are not limited to alcohols, acids (including fatty acids), gases, amino acids, chemicals, and mixtures thereof.

19

The alcohols that may be produced include but are not limited to ethanol, butanol, methanol, propanol, and mixtures thereof.

The acids that may be produced include but are not limited to 2,5-furandicarboxylic acid, itaconic acid, levulinic acid, succinic acid, lactic acid, malic acid, citric acid, acrylic acid, fumaric acid, hydroxypipionic acid, acrylic acid, and mixtures thereof.

The chemicals that may be produced include but are not limited to glycerol, 3-hydropropoionic acid, 2,5-dimethylfuran (DMF), 5-hydroxymethyl furfural (HMF), furfural, aldehydes, amines, terephthalic acid, hexamethylenediamine, isoprene, polyhydroxyalkanoates, 1,3-propanediol, or mixtures thereof.

The gases that may be produced include but are not limited to methane, ethane, CO, CO<sub>2</sub>, H<sub>2</sub>, or mixtures thereof.

## EXAMPLES

### Example 1

#### Enzymatic Hydrolysis of Cotton Textile

Cotton textiles were cut, milled, and then mechanically refined with a PFI mill at 5,000, 10,000, or 20,000 rev. A control was used of no refining. The pretreated cotton textile then underwent enzymatic hydrolysis at 50° C., pH=5.2, and an enzyme load up to 5 FPU/g cotton.

An FPU is a standard way to express enzyme dosage and its ability to convert 50 g of cellulose filter paper into 2.0 mg glucose in 60 minutes. Adney, B. and Baker, J. "Measurements of Cellulase Activities," *NREL Laboratory Technical Report NREL/TP-510-42628*, 2008.

The inventors observed a surprising improvement in the efficiency of cotton conversion (e.g., fibers converted to sugars) with an increase in the intensity of the PFI pretreatment. The more intense PFI pretreatment resulted in shorter fiber lengths and increased percentage of fines by weight. The inventors found a yield increase of 60% from 28% with no refining (control) versus 90% with PFI pretreatment at 10,000 rev. FIG. 2. This demonstrates that the PFI pretreatment lead to an unexpected improvement in cotton textile hydrolysis. See also FIGS. 3-6. Enzymatic hydrolysis experiments were performed at different residence times (24, 48 and 96 h). In all of the cases, PFI mechanical refining highly improved cotton conversion.

The enzymatic hydrolysis experiments were performed at different enzyme charges, for example 4, 5, and 6 FPU/OD grams.

The enzymatic hydrolysis experiments were performed at 5% of cotton content (e.g., 5% of consistency or 5% (w/w) of solid content).

All publications (e.g., Non-Patent Literature), patents, patent application publications, and patent applications mentioned in this specification are indicative of the level of skill of those skilled in the art to which this invention pertains. All such publications (e.g., Non-Patent Literature), patents, patent application publications, and patent applications are herein incorporated by reference to the same extent as if each individual publication, patent, patent application publication, or patent application was specifically and individually indicated to be incorporated by reference.

The invention claimed is:

1. A method of pretreating cotton-containing textile material comprising refining the cotton-containing textile material in a PFI mill for between about 2,000 and 20,000 revolutions,

20

wherein the method does not comprise a pretreatment step that requires neutralization from use of an acid or base, recovery of any solvent, or rinsing steps necessitated from a pretreatment that requires components to be removed before hydrolysis and/or fermentation.

2. The method of claim 1, wherein the method further comprises pretreatment comprising mechanical pretreatment, chemical, enzymatic pretreatment, or a combination thereof.

3. The method of claim 2, wherein the mechanical pretreatment is substantially free of the use of chemicals.

4. The method of claim 2, wherein the mechanically pretreated cotton-containing textile material comprises between about 1% and 50% fines by weight.

5. The method of claim 2, wherein the fiber length LWL (mm) of the mechanically pretreated cotton-containing textile material is between about 0.1 mm and 2.00 mm.

6. The method of claim 2, wherein the Canadian Standard 20 Freeness (CSF) of mechanically pretreated cotton-containing textile material is between about 100 and 900 CSF milliliters.

7. The method of claim 2, wherein the mechanically pretreated cotton-containing textile is in the form of a powder.

8. The method of claim 2, wherein a Wiley Mill is used for the cutting step.

9. The method of claim 2, wherein the mechanical pretreatment is performed before decolorization of the cotton-containing textile material.

10. The method of claim 1, wherein the method further comprises shredding the cotton-containing textile material, cutting the cotton-containing textile material, and milling the cotton-containing textile material prior to refining the cotton-containing textile material in PFI mill.

11. The method of claim 1, wherein a solvent is added to the cotton-containing textile material prior to refining in a PFI mill.

12. The method of claim 11, wherein the solvent is water.

40 13. The method of claim 11, wherein the solvent is added before, during, or both before and during refining.

14. The method of claim 1, wherein the method further comprises enzymatic hydrolysis of the pretreated cotton-containing textile material to produce a hydrolysate.

45 15. The method of claim 1, wherein the method further comprises decolorizing the cotton-containing textile material.

16. The method of claim 15, wherein the decolorizing step comprises bleaching.

50 17. The method of claim 1, wherein the method further comprises adding Cu<sup>2+</sup>.

18. The method of claim 1, wherein the method further comprises adding Fe<sup>2+</sup>.

19. The method of claim 1, wherein the level of refining 55 is between about 2,000 and 20,000 PFI revs.

20. The method of claim 1, wherein the method further comprises subjecting the pretreated cotton-containing textile material to hydrolysis to produce a hydrolysate.

60 21. The method of claim 20, wherein the hydrolysis comprises enzyme hydrolysis comprising the addition of at least one hydrolytic enzyme.

22. The method of claim 21, wherein the enzyme hydrolysis comprises the addition combination of a cellulase and a β-glucosidase.

65 23. The method of claim 20, wherein the method further comprises subjecting the hydrolysate to fermentation to produce an end product.

24. The method of claim 23, wherein the end product produced by fermentation comprises alcohols, sugar alcohols, acids, fatty acids, gases, amino acids, chemicals, and mixtures thereof.

25. The method of claim 1, wherein the method does not 5 comprise a step that requires the use of an acid.

26. The method of claim 1, wherein the cotton-containing textiles comprise cotton, cotton-blend garments, cotton-polyester blend garments, or mixtures thereof.

27. A method of processing cotton-containing textile 10 material comprising

- (a) shredding the cotton-containing textile material;
  - (b) cutting the cotton-containing textile material;
  - (c) milling the cotton-containing textile material;
  - (d) refining the cotton-containing textile material in a PFI 15 mill for between about 2,000 and 20,000 revolutions;  
and
  - (e) subjecting the cotton-containing textile material to hydrolysis to produce a hydrolysate,
- wherein the method does not comprise a pretreatment 20 step that requires neutralization from use of an acid or base, recovery of any solvent, or rinsing steps necessitated from a pretreatment that requires components to be removed before hydrolysis and/or 25 fermentation.

28. The method of claim 27, wherein the cotton-containing textiles comprise cotton, cotton-blend garments, cotton-polyester blend garments, or mixtures thereof.

\* \* \* \* \*